

## UNITED STATES PATENT OFFICE

2,345,580

## STABILIZATION OF MINERAL OILS

Loran O. Buxton, Belleville, N. J., assignor to National Oil Products Company, Harrison, N. J., a corporation of New Jersey

No Drawing. Application June 21, 1941,  
Serial No. 399,213

13 Claims. (Cl. 252—52)

This invention relates in general to the stabilization of mineral oils, and more particularly to the treatment of mineral oils used for lubricating purposes, as constituents of greases, as transformer oils, for pharmaceutical purposes, and for other purposes for which mineral oils are adapted so as to inhibit oxidative changes which tend to take place therein.

It is well known that lubricating oils, etc., frequently undergo deteriorative changes on storage or on being heated or exposed to light. This deterioration is due to the presence of components in the oils which change in composition as a result of various factors. Although there is some disagreement concerning the exact mechanism of these various changes, it is somewhat generally agreed that the deterioration is a result of oxidative changes, and that these changes are affected by the nature of the materials with which the oil comes in contact. As a result of these oxidative changes, sufficient amounts of deleterious products may be formed as to render the oil unsafe for future use. Oxidation of the oil may produce organic acids which tend to react with any metal with which the oil is in contact and produce metallic soaps that are insoluble in the oil. Also various oxidation products of the oil may undergo polymerization or condensation to produce materials insoluble in the oil. Any appreciable formation of these various deleterious substances may so affect the properties of the oil so that it may no longer be efficiently used. In some cases only very minute quantities of oxygen are required to promote undesirable but extensive reactions.

In view of the foregoing and other disadvantages inherent in the use and storage of mineral oils, much work has been done in an attempt to develop various compounds and materials which may be added to mineral oils and effectively protect them from deteriorative changes. Although some of these additives have proved to have some beneficial action, many of them have not been entirely satisfactory.

In carrying out experiments relating to the solvent extraction of fatty materials, I have found that by treating natural antioxidant-containing fatty materials with certain types of organic solvents, highly potent extracts containing the majority of the natural antioxidants of the fatty material concentrated therein may be obtained. Thus I have found that a highly potent antioxidant extract may be obtained from a natural antioxidant-containing vegetable or fish oil by contacting said oil with a suitable sol-

vent at room temperature or above such that at least the major portion of the oil is miscible with the solvent and then cooling the mixture to a temperature within the range of 0° C. to —70° C. whereby a solvent layer containing the desired antioxidant extract separates. Among the solvents which were found to be particularly suitable for use in this process are those listed in the table below:

10

*Table I*

1. Aliphatic and alicyclic monohydroxy alcohols containing from 3 to 6 carbon atoms.
  2. Esters formed by the reaction of aliphatic and alicyclic alcohols with aliphatic monocarboxylic acids, said esters containing not more than 8 carbon atoms.
  3. Aliphatic and alicyclic aldehydes containing not more than 6 carbon atoms.
  4. Aliphatic ketones containing not more than 6 carbon atoms.
- It will be noted that these preferred solvents are all liquid organic compounds having the properties of being substantially miscible with fatty oils at temperatures above room temperature and partially immiscible therewith at temperatures substantially below room temperature; experiments in this connection have shown that solvents of this class may be used generally in
- 25 the process hereinabove described. This process is more fully described and claimed in my copending application Serial No. 351,909, filed August 8, 1940. I have also found that highly potent antioxidant extracts may be obtained
- 30 from natural antioxidant-containing oil-bearing solids, e. g., oil-bearing wheat germ meal, corn germ meal, soybean meal, fish meals, etc., by treating these materials with solvents by a process similar to that of application Serial No.
- 35 351,909. The latter process is more fully described and claimed in copending application Serial No. 397,547, filed June 11, 1941. For further information concerning these processes, reference may be had to the above-identified applications.

It is an object of this invention to provide a process for treating mineral oils so as to retard the development of oxidative changes therein.

A more specific object of this invention is to provide mineral oils, particularly lubricating oils, of improved stability.

I have found that the above and other objects of the invention may be realized by the addition to a mineral oil of a relatively small amount of a natural antioxidant concentrate

produced in accordance with either of the hereinabove identified inventions, or an antioxidant concentrate similar to those produced by the aforementioned processes, but produced by other processes.

Any mineral oil or material containing a mineral oil subject to deteriorative oxidative changes may be treated by the process of my invention. Thus mineral oils used for lubricating purposes, greases containing mineral oil, mineral oils used as transformer oils, white mineral or Russian oils used for pharmaceutical purposes, i. e., oils such as "Nujol," etc., may all be protected from oxidative changes by the incorporation therein of the natural antioxidant concentrates. My antioxidant materials are particularly desirable for treating pharmaceutical mineral oils which are fortified with vitamin products such as vitamin A or other fat-soluble vitamins, as the antioxidant materials in addition to protecting the mineral oil from deteriorative oxidative changes will also quite effectively protect the vitamins from deterioration and oxidation.

It is preferred to use antioxidant concentrates produced from either soybean oil, wheat germ oil, corn germ oil, cottonseed oil, corn oil, sesame oil, etc., or concentrates produced from either oil-bearing wheat germ meal, oil-bearing corn germ meal, oil-bearing soybean meal, etc., or antioxidant concentrates produced from any mixtures of these oils or oil-bearing meals; however, it is to be understood that similar antioxidant fractions from any animal or vegetable oil or meal may be used. Furthermore, this invention also covers the use of antioxidant concentrates similar to those produced by the processes of the two hereinabove identified inventions, but produced by other processes.

In carrying out the process of the invention, a relatively small amount of a natural antioxidant concentrate may be admixed with the mineral oil which it is desired to treat. The amount of antioxidant fraction which is added will depend upon the oil to be treated, the type of deterioration to be prevented, etc. In most cases amounts as low as 0.1% to 0.01% of the weight of the oil to be treated or even lower are sufficient. Obviously the amounts which may be used are not limited to those which are cited as being useful. One skilled in the art will naturally vary the amounts used so as to obtain the optimum results.

The antioxidant concentrates used in the process of my invention may well be used alone for improving the stability of mineral oils; however, if desired, they may be used in combination with other additives which may be incorporated into mineral oils for inhibiting deteriorative oxidative changes. Compounds which may be used in admixture with the natural antioxidant concentrates of my invention include hydroxy compounds, such as phenolic derivatives, naphthols, etc.; nitrogen compounds, including naphthylamines, aniline derivatives, etc.; sulfur compounds as typified by disulfides, thioethers, etc.; and other compounds useful for improving the stability of mineral oils.

As yet the exact chemical composition of the natural antioxidant concentrates used in the process of my invention has not been determined. However, it appears that these antioxidant compositions are not composed of just one or two antioxidant principles, but rather are complex

mixtures containing several antioxidant principles. Because of the complexity of these concentrates, they are of particular value in that they are thus adapted to protecting mineral oils from more than one type of deteriorative oxidative change.

This application is a continuation-in-part of copending application Serial No. 397,547, filed June 11, 1941.

Since certain changes in carrying out the above process and certain modifications in the composition which embody the invention may be made without departing from its scope, it is intended that all matter contained in the above description shall be interpreted as illustrative and not in a limiting sense.

It is also to be understood that the following claims are intended to cover all the generic and specific features of the invention herein described and all statements of the scope of the invention, which as a matter of language, might be said to fall therebetween; and that they are intended to be inclusive in scope and not exclusive, in that if desired, other materials may be added to my novel composition of matter herein claimed without departing from the spirit of the invention. Particularly it is to be understood that in said claims, ingredients or components recited in the singular are intended to include compatible mixtures of said ingredients wherever the sense permits.

Having described my invention, what I claim as new and desire to secure by Letters Patent is:

1. A mineral oil stabilized by the presence therein of a natural antioxidant concentrate prepared by contacting a natural antioxidant-containing material selected from the group consisting of vegetable oils and vegetable oil-bearing solids at a temperature above room temperature with a solvent selected from Table I, cooling the mass to a temperature within the range of 0° C. to -70° C. whereby layers are formed, separating the solvent layer from the insoluble residue and removing the extracted natural antioxidant concentrate from the solvent.

2. A mineral oil stabilized by the presence therein of a natural antioxidant concentrate prepared by contacting a natural antioxidant-containing material selected from the group consisting of vegetable oils and vegetable oil-bearing solids at a temperature above room temperature with isopropanol, cooling the mass to a temperature within the range of 0° C. to -70° C. whereby layers are formed, separating the isopropanol layer from the insoluble residue and removing the extracted natural antioxidant concentrate from the isopropanol.

3. A lubricating oil stabilized by the presence therein of a natural antioxidant concentrate prepared by contacting a natural antioxidant-containing material selected from the group consisting of vegetable oils and vegetable oil-bearing solids at a temperature above room temperature with a solvent selected from Table I, cooling the mass to a temperature within the range of 0° C. to -70° C. whereby layers are formed, separating the solvent layer from the insoluble residue and removing the extracted natural antioxidant concentrate from the solvent.

4. A lubricating oil stabilized by the presence therein of a natural antioxidant concentrate prepared by contacting a natural antioxidant-containing material selected from the group consisting of vegetable oils and vegetable oil-bearing solids at a temperature above room temperature

with isopropanol, cooling the mass to a temperature within the range of 0° C. to -70° C. whereby layers are formed, separating the isopropanol layer from the insoluble residue and removing the extracted natural antioxidant concentrate from the isopropanol.

5. White mineral oil stabilized by the presence therein of a natural antioxidant concentrate prepared by contacting a natural antioxidant-containing material selected from the group consisting of vegetable oils and vegetable oil-bearing solids at a temperature above room temperature with a solvent selected from Table I, cooling the mass to a temperature within the range of 0° C. to -70° C. whereby layers are formed, separating the solvent layer from the insoluble residue and removing the extracted natural antioxidant concentrate from the solvent.

6. A mineral oil base lubricating grease stabilized by the presence therein of a natural antioxidant concentrate prepared by contacting a natural antioxidant-containing material selected from the group consisting of vegetable oils and vegetable oil-bearing solids at a temperature above room temperature with a solvent selected from Table I, cooling the mass to a temperature within the range of 0° C. to -70° C. whereby layers are formed, separating the solvent layer from the insoluble residue and removing the extracted natural antioxidant concentrate from the solvent.

7. A transformer oil stabilized by the presence therein of a natural antioxidant concentrate prepared by contacting a natural antioxidant-containing material selected from the group consisting of vegetable oils and vegetable oil-bearing solids at a temperature above room temperature with a solvent selected from Table I, cooling the mass to a temperature within the range of 0° C. to -70° C. whereby layers are formed, separating the solvent layer from the insoluble residue and removing the extracted natural antioxidant concentrate from the solvent.

8. A mineral oil stabilized by the presence therein of a natural antioxidant concentrate prepared by contacting a natural antioxidant-containing wheat germ oil at a temperature above room temperature with a solvent selected from Table I, cooling the mass to a temperature within the range of 0° C. to -70° C. whereby layers are formed, separating the solvent layer from the insoluble residue and removing the extracted natural antioxidant concentrate from the solvent.

9. A mineral oil stabilized by the presence therein of a natural antioxidant concentrate prepared by contacting a natural antioxidant-containing corn germ oil at a temperature above room temperature with a solvent selected from Table I, cooling the mass to a temperature within the range of 0° C. to -70° C. whereby layers are formed, separating the solvent layer from the insoluble residue and removing the extracted natural antioxidant concentrate from the solvent.
10. A mineral oil stabilized by the presence therein of a natural antioxidant concentrate prepared by contacting a natural antioxidant-containing soybean oil at a temperature above room temperature with a solvent selected from Table I, cooling the mass to a temperature within the range of 0° C. to -70° C. whereby layers are formed, separating the solvent layer from the insoluble residue and removing the extracted natural antioxidant concentrate from the solvent.
11. A mineral oil stabilized by the presence therein of a natural antioxidant concentrate prepared by contacting a natural antioxidant-containing wheat germ oil at a temperature above room temperature with isopropanol, cooling the mass to a temperature within the range of 0° C. to -70° C. whereby layers are formed, separating the isopropanol layer from the insoluble residue and removing the extracted natural antioxidant concentrate from the isopropanol.
12. A mineral oil stabilized by the presence therein of a natural antioxidant concentrate prepared by contacting a natural antioxidant-containing corn germ oil at a temperature above room temperature with isopropanol, cooling the mass to a temperature within the range of 0° C. to 70° C. whereby layers are formed, separating the isopropanol layer from the insoluble residue and removing the extracted natural antioxidant concentrate from the isopropanol.
13. A mineral oil stabilized by the presence therein of a natural antioxidant concentrate prepared by contacting a natural antioxidant-containing soybean oil at a temperature above room temperature with isopropanol, cooling the mass to a temperature within the range of 0° C. to -70° C. whereby layers are formed, separating the isopropanol layer from the insoluble residue and removing the extracted natural antioxidant concentrate from the isopropanol.

LORAN O. BUXTON.

CERTIFICATE OF CORRECTION.

Patent No. 2,345,580.

April 4, 1944.

LORAN O. BUXTON.

It is hereby certified that error appears in the printed specification of the above numbered patent requiring correction as follows: Page 2, first column, line 30, for "metal" read --meal--; page 3, second column, line 37, claim 12, for "70° C." read -- -70° C. --; and that the said Letters Patent should be read with this correction therein that the same may conform to the record of the case in the Patent Office.

Signed and sealed this 23rd day of May, A. D. 1944.

Leslie Frazer

(Seal)

Acting Commissioner of Patents.

CERTIFICATE OF CORRECTION.

Patent No. 2,345,580.

April 4, 1944.

LORAN O. BUXTON.

It is hereby certified that error appears in the printed specification of the above numbered patent requiring correction as follows: Page 2, first column, line 30, for "metal" read --meal--; page 3, second column, line 37, claim 12, for "70° C." read -- -70° C. --; and that the said Letters Patent should be read with this correction therein that the same may conform to the record of the case in the Patent Office.

Signed and sealed this 23rd day of May, A. D. 1944.

Leslie Frazer

(Seal)

Acting Commissioner of Patents.